

# UNITED STATES PATENT OFFICE.

HANS GOLDSCHMIDT AND OTTO WEIL, OF ESSEN-ON-THE-RUHR, GERMANY, ASSIGNEES  
TO GOLDSCHMIDT THERMIT COMPANY, OF NEW YORK, N. Y., A CORPORATION OF  
NEW YORK.

## TITANIUM ALLOYS AND METHOD OF PRODUCING THE SAME.

1,136,670.

Specification of Letters Patent.

Patented Apr. 20, 1915.

No Drawing. Original application filed October 19, 1910, Serial No. 587,857. Divided and this application filed October 29, 1912. Serial No. 728,451.

*To all whom it may concern:*

Be it known that we, HANS GOLDSCHMIDT and OTTO WEIL, subjects of the King of Prussia, German Emperor, and residents of Essen-on-the-Ruhr, in the Province of the Rhine, German Empire, have jointly invented certain new and useful Improvements in Titanium Alloys and Methods of Producing the Same, of which the following is a specification.

Numerous experiments have shown that it is possible by an addition of titanium to improve considerably the quality of steel and cast-iron. The addition of titanium in a metallic state has been attempted, but on account of the bad alloying qualification, the high melting point and the small specific weight of this metal, the results obtained from such attempts have been entirely unsatisfactory, and because of this experts have been of opinion that in order to obtain good results it is necessary to make use, instead of pure titanium, of an iron-titanium-alloy containing only from 10% to 15% of titanium. In many cases, however, it would have been preferable, to add an iron-titanium-alloy containing a high percentage of titanium, but the same objections have been raised to the use of such an alloy as to the employment of metallic titanium, the objection in each case being to the use of a high percentage of titanium.

As a result of our experiments we have found, as set forth in our original application Ser. No. 587,857, filed Oct. 19, 1910, of which this application is a division, that an alloy containing a higher percentage of titanium than has been employed heretofore may be used to advantage in baths of steel and cast-iron if aluminum is added as a third element, in which case we employ an iron-titanium-aluminum-alloy. By using such an alloy as this, with a higher percentage of titanium than has heretofore been employed, the purification of metallic baths, such for example as baths of steel or cast-iron, (by fixing the nitrogen and de-oxi-

dizing and removing the sulphur) is greatly facilitated. The action takes place much more quickly than when an alloy is used containing only from 10% to 15% of titanium. In practice it has been found advisable to use alloys containing from 15% to 35% of titanium and a quantity of aluminum amounting to about 10% of the titanium present, that is to say, 1.5% to 3.5% of aluminum. The alloy may, however, contain a greater percentage of aluminum which in some cases seems advisable.

One of the principal advantages resulting from the addition of the aluminum is that the melting point of the titanium alloy is lowered while the alloying qualification is considerably increased.

Iron-titanium-aluminum alloys suitable for the purpose herein described and of any desired composition may be easily produced by the aluminothermic process. These alloys also have the further advantage of being free from carbon.

An alloy containing from 24% to 25% of titanium and about 3% of aluminum has proved to be very useful.

What we claim is:

1. As a new product, an alloy of ferrotitanium with aluminum containing at least 15% of titanium and in which the aluminum present is at least 10% of the titanium.

2. As a new product, an alloy of iron, titanium and aluminum containing approximately 24% of titanium and approximately 3% of aluminum.

3. As a new product, an alloy of iron, titanium and aluminum containing at least 15% of titanium and at least 1.5% of aluminum.

In witness whereof we have hereunto set our hands in the presence of two witnesses.

HANS GOLDSCHMIDT. [L. S.]  
OTTO WEIL. [L. S.]

In the presence of—

HELEN NUFER,  
ALBERT NUFER.